

Patented May 7, 1929.

1,712,251

# UNITED STATES PATENT OFFICE.

NARAINA DAS CHOPRA AND FREDERICK JOHN BULLEN, OF WESTMINSTER, LONDON, ENGLAND.

## MANUFACTURE OF ROLLED-STEEL MEMBERS.

No Drawing. Application filed December 10, 1926, Serial No. 154,027, and in Great Britain January 2, 1926.

This invention relates to the manufacture of rolled steel members, and for the sake of convenience will be described by reference to the manufacture of steel rails as typifying rolled steel members. It is to be understood, however, that the invention is not limited to the manufacture of steel rails but is applicable to the manufacture of any form of rolled steel member.

10 In the ordinary manufacture of steel rails there occurs a zonic heterogeneity of structure which may be said to be characterized by the presence of three zones, namely, a central zone of pearlitic nature, an outer zone of soft decarburized steel, and an intermediate zone of high-carbon steel. This zoning of structure is generally accompanied by a state of internal instability, and has been found to be mainly responsible for the 20 faults commonly experienced in rails, of corrugation and excessive wear and tear in use.

It is known to be possible to remove from steel defects of the kind referred to above, 25 by annealing, i. e. by a treatment comprising heating the steel to a high temperature and thereafter allowing the metal to cool slowly. Such treatment, however, is generally associated with the disadvantage of 30 producing softening of the steel; it does not eliminate from the structure of the steel the aforesaid zonic heterogeneity, and, further, it leads to the formation of scale, with an accompanying loss of steel by weight.

35 According to the present invention, a process of manufacture of rolled steel members is characterized in this that the completely formed member is submitted to a heat-treatment which comprises heating the member from a temperature below the lowest 40 change-point of the metal to a temperature above (e. g. 50° C. above) the highest change-point, cooling gradually to a temperature somewhat below (e. g. 50° C. below) the lowest change-point, and thereafter more 45 rapidly cooling, for example, by allowing the member to cool spontaneously in the atmosphere. By "highest change point" and "lowest change point" we mean the highest 50 and lowest critical points on heating and cooling, respectively. In the claims these critical points have been designated, respectively, as  $A_c$  and  $A_r$ .

The effect of the special heat-treatment

characterizing this invention is to remove 55 the aforesaid structural defects, or, according to circumstances, materially to reduce them. The process of this invention may be applied as a final heat-treatment of a rolled steel member which has been subjected 60 to the heat-treatment described in the specification of our British Letters Patent No. 271,530 of 1927, in the event of said heat-treatment failing to result in complete elimination or sufficient reduction of the said 65 defects.

Preferrably, the high temperature heat-treatment of the member is effected in the presence of an oxidation inhibitor, by which is meant a solid material which is non-fusible 70 at the temperature employed in the heat-treatment and the action of which, through chemical affinity of the material towards the deleterious furnace gases, is to protect the metal from oxidation or substantially to reduce 75 the degree thereof. Examples of oxidation inhibitors are alkaline earth oxides, such as lime; infusible readily oxidizable materials in a condition to present to the gases a large surface relatively to the area 80 of the exposed surface of the member under heat-treatment, for example shavings or turnings of an oxidizable metal such as steel; and carbonaceous material such as an exhausted carburizing mixture, boiler ash or 85 producer ash, containing an adequate proportion (for example at least 10%) of combustible carbon.

By an exhausted carburizing mixture is meant a carburizing mixture which has been 90 used to such an extent as to render it unsuitable for further use in carburizing. A suitable carburizing mixture which, when exhausted, has been found to be utilizable according to the present invention consists 95 of three parts of powdered beech charcoal and two parts each of powdered horn charcoal and powdered animal charcoal. The boiler ash or producer ash may be of the type which usually contains from 5 to 15 100 per cent of carbon.

The use in heat treatment of steel of a mixture of alkaline earth oxide and an appropriate carbonaceous material containing free carbon such as an exhausted carburizing reagent, forms the subject of our British Letters Patent 271,606 of 1927, and is claimed herein only in conjunction with the spe-

cific heat treatment which characterizes the present invention.

The degree to which the member is heated above the highest change-point or is allowed gradually to cool below the lowest change-point is a factor to be adjusted according to the nature of the member. Our general experience seems to indicate that such degree may be relatively small. For example, we have attained the advantages aforesaid by heating to approximately 50° C. above the highest change-point and gradually cooling to 100° C. below the lowest change-point. We have found that the degree to which the member should be allowed gradually to cool below the lowest change-point is generally not less than 50° C.

We have frequently found in our work upon steel members that the process of this invention gives specially good results in the case of steel containing a small proportion of a metallic element, such as nickel or cobalt, the presence of which tends to depress the change-points of the steel.

According to a further feature of the invention, therefore, the steel member subjected to the aforesaid special heat-treatment is composed of steel containing a small proportion of a metallic change-point depressant, such, for example, as nickel or cobalt.

The proportion necessary of such element is preferably quite small, for example 1% or less. We have usually found 0.5% to be sufficient. In this connection it will be understood that the advantage in question is secured with steel wherein the nickel or other change-point depressant is present even as an adventitious component.

We have also found that the heat-treatment characteristic of this invention is specially effective in the case of chrome steels; and according to a further feature of the invention the steel member subjected to heat-treatment as above is composed of chrome steel. We have found that with this particular special metal the advantageous effects of the invention are frequently very marked.

The chrome steel from which the member is formed may with further advantage be a chrome steel containing a change-point depressant such as nickel or cobalt.

#### Example I.

An ingot was cast from a steel assaying as follows:

|            | Per cent. |
|------------|-----------|
| Carbon     | 0.62      |
| Silicon    | 0.177     |
| Sulphur    | 0.0355    |
| Phosphorus | 0.04      |
| Manganese  | 0.86      |
| Nickel     | 0.54      |

The tapping temperature was 1520° C.

The teaming temperature (with one inch nozzle) was 1450° C.

The top of the ingot mould was covered during setting with an oxidation inhibitor consisting of an exhausted carburizing mixture.

On stripping, the ingot was coated with a further quantity of the aforesaid oxidation inhibitor. The stripping temperature was 960° C.

The ingot was transferred to the soaking pit, the floor of which was covered to a depth of about three inches with a mixture of lime and boiler ash carrying 15.6 per cent of combustible carbon, the proportion of lime to ash being approximately 40:60, and the sides of which were loosely packed around the ingot, with steel turnings. The space beneath the lids of the pit between the top of the ingot and the roof of the furnace was also filled in with loosely disposed steel turnings suspended from the lids of the pit.

The temperature of the ingot was raised in the soaking pit to 1190° C. whereupon the ingot was transferred at the temperature stated to the cogging mill. The temperature during cogging was 1090° C.

The billet, after cogging, was then subjected without further heat-treatment to rolling operations to form the rail and the finishing temperature of the rail was 995° C.

The completely formed rail was then allowed to cool on the hot-banks to a temperature of approximately 500° C., after which it was heated again in a re-heating furnace to approximately 815° C. and thereafter allowed gradually to cool in this furnace to about 540° C. The rail was then removed from the furnace and allowed to cool spontaneously in the air. The reheating and slow cooling treatment in the furnace was effected in the presence of an oxidation inhibitor similar to that employed in the soaking pit, the furnace being packed with the inhibitor in the same way.

The structure of the rail showed itself to be in a homogeneous pearlitic form and the rail exhibited no sign of a decarburized zone at the surface.

#### Example II.

This is an example of the manufacture of a rail from a chrome steel, the analysis of which was as follows:

|            | Per cent. |
|------------|-----------|
| Carbon     | 0.577     |
| Silicon    | 0.205     |
| Sulphur    | 0.032     |
| Phosphorus | 0.02      |
| Manganese  | 0.74      |
| Chromium   | 0.98      |
| Nickel     | 0.52      |

The operations of pouring, teaming, cog-

ging and rolling were carried out as in the Example I, the temperature of the ingot during cogging being 1090° C. and the finishing temperature after the last roll being 5 995° C. The rail after the last roll was allowed, as in Example I, to cool down on the hot banks to about 500° C. after which it was heated again through the change-points to approximately 815° C. and then 10 cooled slowly in the reheating furnace to about 540° C. At this temperature the rail was removed from the furnace and allowed to cool spontaneously in the air to normal temperature. The reheating furnace contained 15 an oxidation inhibitor as in the case of the furnace of Example I. As in the case of Example I the rail showed no signs of zoning of structure.

It was found that without sacrifice of tensile strength both the elongation and the reduction in area of test piece were very materially increased by the special treatment characteristic of this invention as compared with the effects of ordinary treatment 25 involving a mere hot-bank cooling of the finished rail. The following are the strength figures for the rail:—

Maximum tensile strength ----- 50.36 tons per sq. inch  
30 Elongation on 3" ----- 15.0%  
Reduction in area of test piece----- 31.6%

The corresponding figures for an ordinarily manufactured rail of exactly the same treatment up to and including the last rolling operation and exactly the same analysis, with the exception of the presence of nickel in the steel, were as follows:—

40 Maximum tensile strength ----- 50.48 tons per sq. inch  
Elongation on 3" ----- 2.0%  
45 Reduction in area of test piece----- 2.0%

In addition to the improvement indicated above in the figures for elongation and reduction in area, the rails produced according to the above examples behaved better 50 in a very marked degree in the drop tests. Indeed, the difference in behaviour in the drop tests was even more marked than the improvement shown in the tensile strength tests. In the case of the chrome steel rails 55 manufactured by the ordinary process, nearly every rail broke under the drop test at the second blow, whereas of the rails manufactured according to the present invention the majority stood more than three 60 blows at the drop test without fracture.

Reverting again to the oxidation inhibitors the presence of which as aforesaid is preferable during the heat-treatment which characterizes this invention, the inhibitor 65 may comprise sheets or plates of an oxidiz-

able metal such as iron or steel disposed around the walls of the furnace or beneath the roof thereof or in the gas openings. Alternatively, the steel member to be protected may be enveloped during the heat-treatment in a cage built up of sheets or plates or bars of iron or steel or other readily oxidizable metal. 70

Again, if an alkaline earth oxide such as lime be employed as the oxidation inhibitor 75 it may be employed in powder form or in aqueous suspension or solution. The manner of applying the oxide may be varied according to circumstances and convenience. If the member under heat-treatment is the 80 initial hot ingot, or is in the billet stage or, again, is proceeding through the rolling mills, the oxide may be sprayed or dropped upon the member. On the other hand, if the member is undergoing heat-treatment in 85 a soaking pit, reheating furnace or other furnace, the member may be placed in a bath of powdered lime or like oxide or, a paste of the oxide may be coated upon the member. 90

In some cases it may be found preferable either as an alternative to the aforesaid forms and modes of application of oxidation inhibitor or in conjunction therewith to line the soaking pit or other furnace with dolomite or furnace slag. 95

Lastly, with regard to the oxidation inhibitors, any two or more of the aforesaid forms may be employed conjointly.

It is to be understood that the present invention is applicable to the treatment of a defective rail which has been produced by the ordinary methods of manufacture for the purpose of eliminating the defects. 100

We claim:—

1. A process of treatment of rolled steel members which comprises heating the fully-formed member from a temperature below the lowest change-point of the steel to a temperature slightly above the highest  $Ac_1$  110 change-point by direct contact with furnace gases which have been rendered substantially innocuous towards the steel as regards their oxidizing and decarburizing capacity by treatment with an alkaline earth oxide and a substantially non-carburizing carbon-carrying material as herein defined, cooling gradually to a temperature slightly below the lowest  $Ar$  change-point in the presence of material capable of inhibiting oxidation 115 of the steel, and thereafter allowing the member to finish cooling in an uncontrolled manner. 120

2. A process of treatment of rolled steel members according to claim 1, wherein the relative amounts of the oxide and carbon-carrying material are such that the quantity of oxide is equivalent to from 10% to 50% by weight of the combined quantities of oxide and carbon-carrying material and the 125 130

carbon content of the carbon-carrying material is such that the quantity of free carbon present is equivalent to from 4% to 20% by weight of the aforesaid combined quantities.

5. 3. A process of treatment of rolled steel members according to claim 1, wherein the heating operation is effected in the presence of a false increase of area of oxidizable material provided by a mass of infusible 10 readily oxidizable material, substantially as and for the purpose set forth.

4. A process of treatment of rolled steel members, which comprises heating the fully-formed member by direct contact with hot 15 furnace gases through the Ac change-points of the steel to a temperature of about 50° C. above the highest change-point, in a furnace containing a sufficiency of lime and substantially non-carburizing carbon-carrying material as herein defined to render and maintain the furnace gases substantially innocuous towards the steel as to their oxidizing and decarburizing capacity, ceasing the heating operation and allowing 20 the member to cool gradually to a temperature of about 50° C. below the lowest Ar change-point in the presence of material capable of inhibiting oxidation of the steel, and thereafter allowing the member to 25 finish cooling in an uncontrolled manner.

5. A process of treatment of rolled steel members, which comprises heating the fully-formed member by direct contact with hot furnace gases through the Ac change-points 30 of the steel to a temperature of about 50° C. above the highest Ac change-point, in a furnace containing a mass of infusible readily oxidizable material in a form to provide in the furnace a relatively large 35 false increase of oxidizable surface area exposed to the furnace gases and a sufficiency of lime and substantially non-carburizing carbon-carrying material as herein defined to render and maintain the furnace gases 40 substantially innocuous towards the steel as to their oxidizing and decarburizing capacity, ceasing the heating operation and allowing the member to cool gradually to a temperature of about 50° C. below the lowest Ar change-point in the presence of material 45 capable of inhibiting oxidation of the steel, and thereafter allowing the member to finish cooling in an uncontrolled manner.

6. A process of treatment of rolled steel members according to claim 4, wherein the relative amounts of the lime and carbon-carrying material are such that the quantity of lime is equivalent to from 10% to 50% by weight of the combined quantities 55 of lime and carbon-carrying material and the carbon content of the carbon-carrying material is such that the quantity of free carbon present is equivalent to from 4% to 20% by weight of the aforesaid combined 60 quantities.

7. A process of treatment of rolled steel members, which comprises heating the fully-formed member by direct contact with hot furnace gases through the Ac change-points 70 of the steel to a temperature about 50° C. above the highest Ac change-point, in a furnace containing a sufficiency of lime and substantially non-carburizing carbon-carrying material as herein defined to render and maintain the furnace gases substantially 75 innocuous towards the steel as to their oxidizing and decarburizing capacity, ceasing the heating operation and allowing the member to cool gradually in the furnace and in 80 the presence of the lime and carbon-carrying material to a temperature about 50° C. below the lowest Ar change-point, and thereafter allowing the member to finish 85 cooling in an uncontrolled manner, the relative amounts present of the lime and carbon-carrying material being such that the quantity of lime is equivalent to from 10% to 50% by weight of the combined quantities of lime and carbon-carrying material 90 and the carbon content of the carbon-carrying material is such that the quantity of free carbon present is equivalent to from 4% to 20% by weight of the aforesaid combined 95 quantities.

8. A process of treatment of rolled steel members according to claim 4, wherein the steel of which the member is composed is chrome steel.

9. A process of treatment of rolled steel members according to claim 4, wherein the steel of which the member is composed is chrome steel containing a small proportion of a change-point depressant.

In testimony whereof we have signed our names to this specification.

NARAINA DAS CHOPRA.  
FREDERICK JOHN BULLEN.